

## UNITED STATES PATENT OFFICE

2,602,776

## ELECTROLYTIC METHOD OF WINNING ZINC

Geoffrey J. J. Mould, Flin Flon, Manitoba, Canada, assignor to Hudson Bay Mining and Smelting Co., Limited, Winnipeg, Manitoba, Canada, a corporation of Canada

No Drawing. Application September 7, 1948,  
Serial No. 48,150

3 Claims. (Cl. 204—119)

1

This invention relates to addition agents for electrolytic cells and to the method of obtaining higher current efficiencies by the use of them when metals are plated out of solution. More particularly it relates to a method of obtaining a higher current efficiency when zinc is plated out from zinc electrolytes used in the electrolytic method of winning zinc from ores or other materials.

It is well known in the art of plating metals from electrolytes that the amount of metal deposited by a certain amount of electricity is below the amount to be expected on the basis of Faraday's law. Thus, in the plating of zinc from a zinc sulphate solution as is usual in the electrolytic method of winning zinc the amount of zinc deposited from what may be termed a good commercial electrolyte ranges from 85% to 95% of that calculated according to Faraday's law, the deficiency resulting from the evolution of hydrogen.

The current efficiency obtained in the plating of zinc is of great commercial importance, because of the cost of electric current, more current being required per pound of zinc when the efficiency is low and particularly because when the efficiency is low the zinc is not deposited in a compact sheet but is full of holes. Such zinc is difficult to handle in the stripping and melting operations which follow. Moreover, when the zinc is deposited at low current efficiencies the zinc contains more impurities than is the case where the current efficiencies are high. In the normally known methods of winning zinc electrolytically the zinc obtained is comparatively poor, being rough and porous, and no means has been discovered, so far as is known up to the date of the present invention, to overcome this difficulty.

Various factors have a deleterious effect on current efficiency and the best known and most important is the presence of certain impurities in the electrolyte such as antimony, arsenic, cobalt, iron, nickel, germanium, tin, selenium, tellurium, copper, the platinum metals and, according to some investigators, silicon.

The difficulties above enumerated have been overcome by the present invention according to which an improvement is obtained in the current efficiency of zinc deposition by adding small amounts of rosin soap (a sodium rosin soap), to zinc electrodeposition cells in amounts, of three-quarters of a pound up to ten pounds per ton of cathode zinc to be deposited but normally in amounts of the order of one and a half

2

pounds per ton of cathode zinc to be deposited. The addition of a reagent to an acid zinc electrodeposition cell for the purpose of causing the zinc to become non-wettable, protects the zinc from the acid and a better product is obtained. If a rosin soap is added to the electrolyte, the zinc is rendered resistant to corrosion and the addition of the soap within limits leads to increased current efficiency.

10 In order to illustrate the invention reference is made to the following examples of experiments which have been performed.

Samples of certain oils, waxes and resins, set forth below, were saponified by heating with a 15 solution of sodium hydroxide until reaction had ceased, and then the soap compounds from the resultant mixture were separated by salting out, a method well known in the art of soap-making. To ensure that the material obtained was more 20 or less completely saponified, this same material was again heated together with more sodium hydroxide solution, and the soap compounds again were separated from the resultant mixture by salting out.

25 The product obtained was dried and converted into a water solution such that 100 ml. of solution contained one gram of the dried soap.

The various soaps were tested in zinc electrodeposition cells of a standard type, the cathodes 30 being aluminum, and the anodes lead, spaced so that the surfaces of the electrodes were about one inch part. The current was adjusted so that the cathode current density was about thirty-six amperes per square foot. The feed introduced to the cells at the bottom contained about 35 120 grams per litre of zinc as sulphate solution, and the rate of feed was matched with the rate of zinc deposition, the operation being so carried out that the stripped solution which overflowed at the surface of the electrolyte contained approximately 120 grams per litre of sulphuric acid.

40 Every twenty-four hours the cathode was removed from the cell, and the zinc plated thereon removed and dried and weighed.

45 When soap solutions prepared as already described were added daily to such a cell in the amount of 5 ml. per litre of electrolyte per day, the efficiency of zinc electrodeposition was very noticeably improved.

The details of one set of such tests, in which 50 four cells, such as have been described, were operated together in such a manner that the current passing through all the cells was exactly the same, appear below.

To one cell, referred to as cell No. 1 was added after stripping each day, 5 ml. of soap solution per litre of electrolyte, the soap solution having been prepared from rosin in the manner already described.

Similarly, to cell No. 2 was added after stripping each day, 5 ml. per litre of soap solution prepared from croton oil.

Similarly, again, to cell No. 3 was added after stripping each day, 5 ml. per litre of soap solution prepared from castor oil.

Cell No. 4 was a cell to which no additions were made and it was used in the experiment for comparison purposes.

Each of these cells was operated in exactly the same manner, and the solution fed to each cell was exactly the same, containing, besides zinc sulphate, impurities as found in the electrolyte as fed to the electrodeposition cells in the electro-winning of zinc. A portion of this solution was assayed and the following amounts of certain impurities were found:

Cobalt, 10.3 milligrams per litre.

Arsenic, .05 milligrams per litre.

Antimony, .04 milligrams per litre.

Under these conditions, and over a period of ten days the following results were obtained:

|              | Cell No. 1:<br>Daily addi-<br>tions of 5<br>ml. per litre<br>rosin soap<br>soln. | Cell No. 2:<br>Daily addi-<br>tions of 5<br>ml. per litre<br>croton soap<br>soln. | Cell No. 3:<br>Daily addi-<br>tions of 5<br>ml. per litre<br>castor soap<br>soln. | Cell No. 4:<br>Cell for<br>comparison<br>purposes.<br>No addition. |
|--------------|----------------------------------------------------------------------------------|-----------------------------------------------------------------------------------|-----------------------------------------------------------------------------------|--------------------------------------------------------------------|
| Av. C. E.    | Per Cent<br>74.7                                                                 | Per Cent<br>63.1                                                                  | Per Cent<br>59.3                                                                  | Per Cent<br>40.0                                                   |
| Av. Pb Assay | .0020                                                                            | .0035                                                                             | .0034                                                                             | .0056                                                              |
| Av. Cu Assay | .0008                                                                            | .0007                                                                             | .0008                                                                             | .0008                                                              |
| Av. Cd Assay | .0004                                                                            | .0004                                                                             | .0005                                                                             | .0004                                                              |

The results of other experiments are given hereunder.

| Test<br>No. | Kind of Soap                               | Av.<br>Daily<br>Zinc<br>Yield<br>(gms.) | Per<br>Cent<br>of<br>Pilot<br>Yield | Remarks                                                                  |
|-------------|--------------------------------------------|-----------------------------------------|-------------------------------------|--------------------------------------------------------------------------|
| 1-----      | Toilet or hand soap (common, hand milled). | 162.6                                   | 113.6                               | Fairly good electrolyte                                                  |
|             | Linseed Soap.....                          | 149.6                                   | 104.6                               | Co As Sb mg/1                                                            |
|             | Rosin Soap.....                            | 160.9                                   | 112.3                               | 9.9 .02 .03                                                              |
|             | Pilot.....                                 | 143.0                                   | 100.0                               |                                                                          |
|             | Peanut Soap.....                           | 159.6                                   | 108.0                               |                                                                          |
| 2-----      | Cocoanut Soap.....                         | 154.5                                   | 104.8                               | Fairly good electrolyte                                                  |
|             | Palm Soap.....                             | 162.6                                   | 110.1                               | Co As Sb mg/1                                                            |
|             | Pilot.....                                 | 147.5                                   | 100.0                               | 10.1 .03 .026                                                            |
|             |                                            |                                         |                                     | Switched over to less pure electrolyte about half way through this test. |
|             |                                            |                                         |                                     | Co As Sb mg/1                                                            |
| 3-----      | Beeswax Soap.....                          | 168.0                                   | 164.1                               | 10.3 .05 .04                                                             |
|             | Soyabean Soap.....                         | 146.8                                   | 143.2                               |                                                                          |
|             | Rapeseed Soap.....                         | 132.3                                   | 129.2                               |                                                                          |
|             | Pilot.....                                 | 102.3                                   | 100.0                               |                                                                          |
|             |                                            |                                         |                                     |                                                                          |
| 4-----      | Rosin Soap.....                            | 159.7                                   | 186.0                               | Same feed as used in latter part of previous test.                       |
|             | Croton Soap.....                           | 135.6                                   | 158.0                               |                                                                          |
|             | Castor Soap.....                           | 126.9                                   | 148.0                               |                                                                          |
|             | Pilot.....                                 | 85.8                                    | 100.0                               |                                                                          |

The effect of change of electrolyte can be seen in the last group where an impure electrolyte was used throughout the test and in the next to last test in which rather impure electrolyte was used in the latter part of the test.

Soaps from beeswax which contain palmitic derivatives and melissyl alcohol and soaps from resin were found to give the smoothest plates. The judicious addition of wetting agents has an effect in smoothing the plates.

Suitable ranges and the preferred amounts of various soaps tried are as hereunder:

| 5  | Agent                                                                                                    | Amounts in Pounds per Ton of Cathode Zinc |                  |
|----|----------------------------------------------------------------------------------------------------------|-------------------------------------------|------------------|
|    |                                                                                                          | Suitable Range                            | Preferred Amount |
| 10 | Toilet or hand soap consisting essentially of the sodium salts of palmitic, stearic and oleic acids..... | 0.05 to 5.0                               | 0.5 to 1.0       |
|    | Beeswax soap.....                                                                                        | 0.05 to 5.0                               | 0.5 to 1.0       |
|    | Rosin soap.....                                                                                          | 0.05 to 5.0                               | 0.5 to 1.0       |
|    | Glue with above soaps.....                                                                               |                                           | 0.5              |
|    | Wetting Agents with soaps.....                                                                           |                                           | 0.5              |
|    | Gardinol.....                                                                                            |                                           | 1.0              |

Gardinol is an alkyl sodium sulphate containing the lauryl radical and/or the myristyl radical. Both lauric acid  $C_{12}H_{24}O_2$  and myristic acid  $C_{14}H_{28}O_2$  are normal saturated monobasic acids. The structure of Gardinol may be represented by the formula



where R is the organic radical.

Another agent which may be used is Duponol which is a higher alkyl sulphate made from a mixture of lauryl and oleyl alcohols. Oleic acid is an unsaturated monobasic acid of composition  $C_{18}H_{34}O_2$ .

The smoother zinc sheet obtained with the use of beeswax soap is thought to be due to the alcohol modifying the waterproofing action of the palmitic soap. Therefore the alcohol acts more or less as a wetting agent.

It is not easy to get zinc to plate onto the cathode and to keep it there without its redissolving.

40 A water shedding film of soapy material more or less prevents the acid in the cell from attacking the zinc on the cathode. On the other hand this same film of soapy material may make the process of plating onto the cathode a harder thing to do due to the material acting as an electrical insulation. There are therefore two factors which have to be balanced, one against the other to obtain the maximum yield of zinc. It does not follow therefore that the soap which has the most waterproofing effect is necessarily the best for increasing the current efficiency. The best known soaps at the moment for obtaining the desired results are common rosin soap and beeswax soap. Beeswax soap is relatively expensive as compared with common rosin soap but both give good plates and the purity of the zinc deposited is improved. Used in amounts of one to one and a half pounds per ton of cathode zinc deposited they are very satisfactory.

45 60 The embodiments of the invention in which an exclusive property of privilege is claimed are defined as follows:

1. In a process of winning zinc which comprises electrodepositing zinc from a zinc sulphate electrolyte, the improvement which consists in adding a sodium rosin soap to the zinc sulphate electrolyte in an amount effective to increase the current efficiency.

2. The improvement in a process of winning zinc as defined in claim 1 wherein the amount of sodium rosin soap added to said electrolyte varies between three-quarters of a pound and ten pounds per ton of cathode zinc to be deposited.

3. The improvement in a process of winning zinc as defined in claim 1 wherein the amount

of sodium rosin soap added to said electrolyte is about one and one half pounds per ton of cathode zinc to be deposited.

GEOFFREY J. J. MOULD.

REFERENCES CITED

The following references are of record in the file of this patent:

UNITED STATES PATENTS

| Number    | Name            | Date          |
|-----------|-----------------|---------------|
| 1,876,156 | Thompson et al. | Sept. 6, 1932 |
| 1,895,675 | Mathers         | Jan. 31, 1933 |

| Number      | Name   | Date          |
|-------------|--------|---------------|
| 2,113,517   | Powell | Apr. 5, 1938  |
| 2,389,135   | Brown  | Nov. 20, 1945 |
| 2,389,179   | Brown  | Nov. 20, 1945 |
| 5 2,389,180 | Brown  | Nov. 20, 1945 |

OTHER REFERENCES

Transactions of the American Electrochemical Society, vol. XLV (1924), pages 414, 415, 420, 428.  
 10 Silman: Journal of Electrodepositors' Technical Society, vol. 19 (1943-44), pages 131-134, 141-145.